

Patented Oct. 5, 1926.

1,601,746

# UNITED STATES PATENT OFFICE.

THOMAS TERRELL, OF TEMPLE, LONDON, ENGLAND.

MANUFACTURE OF INCANDESCENT GAS MANTLES.

No Drawing. Application filed November 7, 1925, Serial No. 67,698, and in Great Britain November 21, 1924.

When gas mantles were first manufactured they were produced as follows:—A natural cotton knitted fabric was dipped in a solution of salts (nitrate of thorium with about 1 per cent nitrate of cerium) and dried. The fabric was then burned out with a Bunsen gas flame and left, as a simulacrum of the fabric, a residue of the oxides of the rare earths used. The elementary fibres of the cotton thread being more or less tubular and twisted the oxide residues had a similar form, they were very brittle and being the result of the destructive burning of the nitrates had a more or less volcanic appearance under the microscope. It was subsequently discovered that a ramie fibre had great advantage over cotton in that being more solid and not twisted it produced a better ash and consequently ramie was very generally substituted for cotton but there was this disadvantage that the ramie thread was much coarser than the cotton thread and consequently in the unburned mantle the percentage of organic to inorganic material was much higher; this resulted in the finished mantle being much more porous and coarse in proportion to its actual weight. It had been thought that artificial silk would produce a better mantle than either ramie or cotton but all attempts to use it failed until Plaisetty conceived the idea of denitrating the salts before incineration. This he did by dipping the knitted fabric in the salt solution, drying it, and then dipping it in a solution of ammonia gas, washing out the nitrate of ammonia and drying again, and the result was a mantle composed of cellulose and oxides of the rare earths in solid solution. It was afterwards discovered that cotton could be successfully used in the same way but the defects of the cotton mantle to a very large extent remained. It was generally considered that a mantle say of the size known in the British trade as a "universal inverted mantle" should when finished contain .5 grams of oxides and that its durability and strength depended upon this weight being approximated.

The elementary fibres of the artificial silk heretofore used in the manufacture of mantles were of a thickness equivalent to from 5 to 7 deniers Italian London silk conditioning house measurement (hereinafter referred to as Italian silk measurement) and the thread used to knit the fabric for the man-

ties was from 140 to 200 deniers. This was considered necessary to produce the weight mentioned above of .5 grams per mantle.

I have ascertained that the strength and durability of a mantle does not depend upon a heavy weight of oxides but upon the fineness of the elementary fibres of which it is composed and further that when a very fine fibre is used say of .5 to 3 deniers in thickness they may be spun or thrown to produce a very fine yarn of say 1/100 to 1/80 metric measurement or even less and that when this yarn is knitted and dipped a mantle can be made of the size mentioned containing only .2 to .25 grams weight of oxides and that this mantle is very superior in strength, durability and in light emission to any mantle hitherto manufactured. By "metric measurement" is meant proportion of length to weight. The experiments which I have conducted lead me to the conclusion that if it were possible to knit and form a mantle out of a single strand of cellulose as fine as the fibre of a spider's web and to dip and burn it, there would be produced the strongest and most durable mantle possible in actual use and its light emission would be of the best.

My invention consists in using a lustra cellulose fibre which is made as fine as possible say from .5 to 3 deniers Italian silk measurement in thickness. In practising the invention I prefer to use fibre of 1 denier in thickness and to throw or spin this fibre into yarn of 1/100 to 1/40 metric measurement approximately (preferably 1/80) and to use such yarn in the manufacture of the mantles. If I am making the "universal" mantles I have already referred to I prefer to knit this yarn on a 160 needle machine having a cylinder 9 centimetres in diameter and I knit with 5 rows of stitches to each centimetre. I dip this material conveniently in a 50 per cent solution of the salts and throw out the solution therefrom so that 100 grams dry shall weigh 200-300 grams when impregnated and wet. I dry, denitrate, and dry again. The result will be approximately that 100 grams of the original fabric will give 125-150 grams of impregnated material—calculated chemically dry. A universal mantle of this manufacture in which yarn of 1/80 metric measurement has been used as aforesaid may be made to contain as low

as .25 grams of oxide. A mantle made of this material and in this manner will weigh in both lustra cellulose and thorium oxide just about half that of a mantle made by 5 any process hitherto in vogue and yet will be considerably stronger and more durable and more light emitting.

Another great advantage of the present invention arising from the fact that the elementary fibre of the lustra cellulose is extremely fine, is that the fibre being so fine it is very soft and its texture has the feeling of fine wool in the place of the harsh texture of ordinary artificial silk or of ramie or even 10 natural cotton. The substance when impregnated preserves this softness and the mantles made from it need not be burned off in the factory to get their proper shape—they may be put on rings and sold in that condition. The buyer can place a mantle on his ordinary burner and light it so as to burn out the organic matter and he can then turn on the gas and even at a pressure of 5 cm. of water or less the gas will, acting on this 15 very soft material, blow it out to its proper shape so that it becomes undistinguishable from a mantle burned off at the factory and sold, as it is technically termed, "hard." No soft mantles although many have been sold 20 in that condition have ever before presented this advantage and there is this further advantage that soft mantles made according to the present invention have a fully efficient life of over 2000 hours continuous burning 25 which hitherto no mantle however made has approached. The shrinkage on continuous burning is practically nil and the fibres being so very fine they attain the highest temperature the flame will give and the light emitted 30 is consequently very white.

A soft mantle made according to the invention of the size of a universal inverted mantle as aforesaid would contain about .5 grams of lustra cellulose and .25 to .30 grams 35 of oxide.

In construing this specification 1/40 metric measurement means 40,629 metres per kilogram and 1/100 means 101,573 metres per kilogram and other counts in proportion 40

and 1 denier is estimated to be about 9,141,- 50 000 metres per kilogram—all these measurements are only approximate as it is impossible to spin or throw to such regularity—and "lustra cellulose" means cellulose with a bright translucent appearance and each 55 elementary fibre of which is solid as compared to the structure of natural cotton and further is within the limits of thickness herein specified.

What I claim and desire to secure by Letters Patent of the United States is:—

1. An incandescent gas mantle in which there has been used lustra cellulose the thickness of the elementary fibre of which is within the range of .5 to 3 deniers Italian silk 65 measurement.

2. An incandescent gas mantle in the marketable soft condition having a fabric of lustra cellulose the elementary fibre of which has a thickness within the range of .5 to 3 70 deniers Italian silk measurement.

3. An incandescent gas mantle in which there has been used yarn of a weight not exceeding 1/40 metric measurement and such yarn being composed of lustra cellulose the 75 thickness of the elementary fibre of which is within the range of .5 to 3 deniers Italian silk measurement.

4. An incandescent gas mantle in the marketable soft condition having a fabric of 80 yarn not exceeding 1/40 metric measurement, such yarn being composed of lustra cellulose, the elementary fibre of which has a thickness within the range of .5 to 3 deniers Italian silk measurement.

5. An inverted incandescent gas mantle of the size known in the British trade as a "universal inverted mantle" containing from .25 grams to .30 grams of oxide.

6. An inverted incandescent gas mantle in 85 the marketable soft condition and of the size known in the British trade as a "universal inverted mantle" having a fabric of lustra cellulose of about .5 grams in weight of lustra cellulose and containing from .25 90 to .30 grams of oxide.

THOMAS TERRELL.